

# UNITED STATES PATENT OFFICE.

WILLIAM N. BLAKEMAN, JR., OF NEW YORK, N. Y.

## OIL AND COMPOUND THEREOF.

989,226.

Specification of Letters Patent. Patented Apr. 11, 1911.

No Drawing.

Application filed May 26, 1905. Serial No. 262,375.

*To all whom it may concern:*

Be it known that I, WILLIAM N. BLAKEMAN, Jr., a citizen of the United States, and resident of the borough of Manhattan, in the city, county, and State of New York, have invented certain new and useful Improvements in Oils and Compounds Thereof, which invention is fully set forth in the following specification.

10 The object of this invention is to treat fatty oils in such a manner that, when a pigment is ground therein, a paint will be formed which will dry satisfactorily and be durable and permanent.

15 The invention consists in incorporating with a fatty oil, before a pigment is ground therein, a chlorinated fatty substance, as will now be described in detail and then set forth in the claims.

20 In carrying out my invention I first form a chlorinated fatty agent, and for this purpose may be employed any of the drying fatty oils (such as linseed, hemp, poppy or tung) the non-drying fatty oils (such as 25 cotton, sunflower and corn), the rosin oils, or a constituent or derivative of these substances, such as oleic acid, stearin and stearic acid. I prefer to employ either linseed, tung or rosin oil.

30 Selecting tung oil, as an example, I treat it with chlorin in any manner that shall give a satisfactory product, such as by passing chlorin through the oil, arranged in a tall column; by exposing the oil, in broad 35 surfaces, to the action of chlorin; or by subjecting the oil to any other suitable chlorinating process that will produce a chlorinated agent. After thoroughly washing the product, I introduce any desired proportion

40 of it into the fatty oil to be used as a paint-vehicle, thoroughly commingling and blending the same and then grind in this vehicle the pigment or pigments to be used. I prefer to employ pigments which, ordinary,

45 are deficient in spreading power when ground in oil, such as zinc oxid, zinc sulfid, lead carbonate, lead sulfate, lead sulfite, sublimed lead, barium sulfate or barium carbonate, and have obtained the best results 50 when an oxid or sulfid is used either as a

sole pigment or combined with others, as oxids and sulfids appear to form more satisfactory combinations with the chlorinated agent. For my purpose, a sulfid is the equivalent of an oxid. A drying oil, raw or oxidized, (such as linseed or tung) or a commercial drier, or both, may be added to the compound to accelerate its drying when spread as a paint.

Any of the fatty substances above named 60 may be chlorinated in a manner similar to that described for tung oil, and used in the same way, and hence by the use of the term "chlorinated fatty agent" in this specification and in the claims, I intend to cover the 65 product resulting from chlorinating any of the fatty substances named, or any other equivalent substance which will produce substantially the same ultimate result.

The fatty agent, either before or after being chlorinated, may be oxidized by heating with oxidizers; by introducing a portion of highly oxidized matter soluble in, or miscible with, the oil; by elaidinizing the oil; or by introducing a portion of elaidinized 75 matter soluble in, or miscible with, the oil. And the oil-vehicle, with which the chlorinated fatty agent is incorporated, may also be similarly oxidized if desired. It will be found advantageous in many cases to oxidize 80 either the agent or the vehicle, or both, and in particular when using non-drying oils.

Two or more chlorinated fatty agents may be used, if desired in one vehicle; or any combination of fatty oils, either drying or 85 non-drying, may be used as a vehicle and treated with a chlorinated agent as described. If desired the vehicle, or one or more of the oils of which it is composed, may be slightly chlorinated as described in 90 another application No. 262,374, filed by me herewith. In forming combinations of oils, it will be found of advantage to allow the oils to stand for a few days for "blending."

In most cases I prefer to incorporate in 95 the vehicle, a proportion of tung oil, as its presence appears not only to accelerate the drying of the paint but also to improve the quality of the film.

My invention will be found particularly 100

applicable to the non-drying fatty oils, as such oils when treated with a chlorinated fatty agent and used as a paint-vehicle, either alone or in combination with a drying oil, will form with all those pigments ordinarily deficient in spreading power when ground in oil, a paint-compound which will dry into a smooth and tough film, repellent to the elements and unaffected by climatic changes.

The proportions to be used of oil vehicle, chlorinated fatty agent, and pigment, can be easily regulated in practice and may be considerably varied. If an oxid or sulfid be employed as a pigment, it may be used in such proportion as to form the sole pigment; or, only a small proportion—say from 1 to  $1\frac{1}{2}$  per cent.—may be used, with from one-half of one per cent. to  $1\frac{1}{4}$  per cent. of a chlorinated agent in the vehicle, and the remaining portion of the pigment may be of any of the metallic salts above named. If sublimed lead be used as a pigment, I prefer to combine with it a proportion of free zinc oxid. A compound of 100 parts of linseed oil, one per cent. of chlorinated tung oil as an agent, 200 parts of sublimed lead, and 20 parts of zinc oxid will, with the usual quantity of liquid drier, form a satisfactory mixture when spread as a paint. So also will a compound of 100 parts of linseed oil, one per cent. of chlorinated tung-oil-agent, 200 parts of lead carbonate, and 20 parts of zinc oxid. Iron oxids and the ferruginous earths, when ground in a non-drying fatty oil treated with a chlorinated fatty agent, will form cheap and permanent paints.

Heat, pressure and agitation may be employed whenever deemed necessary.

I am aware that it has been proposed heretofore, to incorporate with fatty oils, chlorid of sulfur, either alone or in solution in a hydrocarbon, the alleged result being the production of a sulfo-chlorinated fatty oil. Such processes I expressly disclaim as foreign to my invention. The main object sought to be accomplished in these processes was the sulfurizing of the fatty oil, and the chlorination, if effected at all, was merely incidental; whereas, in my invention the chlorination of the fatty oil is the essential feature, and sulfurizing would be not only unnecessary but objectionable. I am also aware that it has been proposed to decolorize or bleach oils, and also to clarify oils, by the use of various hypochlorites; but such processes I also expressly disclaim, as they will not produce a chlorinated oil. My experiments have shown that the only satisfactory way of chlorinating the fatty substances used as agents in my invention is by contact with free chlorin, as hereinbefore described; and chlorination in this way, instead of

bleaching the fatty substance has a darkening effect upon it. In none of these prior processes, is a chlorinated fatty agent incorporated in a fatty oil; and I am not aware that any one, prior to my invention, has first formed a chlorinated fatty agent by treating a fatty substance with free chlorin and then incorporated this chlorinated fatty agent in a fatty oil, the result being the production of an oil-vehicle which is adapted for use, with all the pigments named, in the formation of very durable and permanent compounds. And the advantage secured by incorporating in commercial oil a chlorinated fatty agent, instead of chlorinating the whole mass of commercial oil, is that, by regulating the quantity of chlorinated fatty agent used, the commercial oil may be brought into condition for use with any of the pigments named, which pigments, by reason of differences in chemical and physical properties, require different proportions of chlorinated agent, in the vehicle, in order that the best results may be produced; whereas, if the whole mass of commercial oil vehicle were chlorinated by treatment with chlorin, many vehicles, each exhibiting a different degree of chlorination, would have to be put upon the market to meet the requirements of the different pigments. This marked advantage of my invention has been described above in the use of a chlorinated tung-oil-agent, and it becomes even more apparent, from an economical standpoint, if chlorinated stearins be used as agents. From 5 to 10 per cent. of any of the stearins, chlorinated by contact with free chlorin, as herein described; and then incorporated in commercial linseed or other oil, will cause the latter to form satisfactory compounds with all the pigments usually deficient in spreading and drying properties.

Having thus fully described my invention, I claim:—

1. As a new composition of matter, a compound or mixture of a fatty oil and a chlorinated fatty substance, the fatty oil being in excess.
2. A compound or mixture of an oil and chlorinated tung-oil.
3. As a new composition of matter, a compound or mixture of an oxidized fatty oil and a chlorinated fatty substance, the fatty oil being in excess.
4. A compound or mixture of an oxidized oil and chlorinated tung oil.
5. As a new composition of matter, a compound or mixture of a non-drying fatty oil and a chlorinated fatty substance, the fatty oil being in excess.
6. A compound or mixture of a non-drying fatty oil and chlorinated tung oil.
7. As a new composition of matter, a com-

pound or mixture of an oxidized non-drying fatty oil, and a chlorinated fatty substance, the fatty oil being in excess.

8. A compound or mixture of an oxidized non-drying fatty oil; and chlorinated tung oil.

9. The process herein described, which

consists in first chlorinating a fatty substance by contact with free chlorin, and then incorporating it in a fatty oil.

WM. N. BLAKEMAN, JR.

Witnesses:

FRANCIS P. REILLY,

MABEL O. FAHNESTOCK.